



# United States Patent [19]

Kageyama

[11] Patent Number: 5,356,573

[45] Date of Patent: Oct. 18, 1994

[54] SNOW SKI BASE MATERIAL AND SKI BASE MANUFACTURE

[75] Inventor: Norihiro Kageyama, Hamamatsu, Japan

[73] Assignee: Yamaha Corporation, Hamamatsu, Japan

[21] Appl. No.: 980,236

[22] Filed: Nov. 23, 1992

Related U.S. Application Data

[62] Division of Ser. No. 640,860, Jan. 14, 1991, Pat. No. 5,189,130.

[30] Foreign Application Priority Data

Jan. 19, 1990 [JP] Japan ..... 2-9550

[51] Int. Cl.<sup>5</sup> ..... H05B 6/00

[52] U.S. Cl. ..... 264/25; 264/320; 264/322; 264/158; 528/503

[58] Field of Search ..... 264/319, 320, 322, 25, 264/158; 528/503

[56] References Cited

U.S. PATENT DOCUMENTS

3,944,536 3/1976 Luptun et al. ..... 528/503  
5,037,928 8/1991 Li et al. ..... 526/352

FOREIGN PATENT DOCUMENTS

0186995 7/1986 European Pat. Off. .

0340211 11/1989 European Pat. Off. .

61-82772 4/1986 Japan .

61-217980 9/1987 Japan .

OTHER PUBLICATIONS

PTO Translation of JP 61-82772.

Renfrew and Morgan, Polythene (The Technology and Uses of Ethylene Polymers). First Ed., pp. 91-118.

French Search Report dated Sep. 21, 1992.

Primary Examiner—Joseph L. Schofer

Assistant Examiner—David Wu

Attorney, Agent, or Firm—Burns, Doane, Swecker & Mathis

[57] ABSTRACT

A high performance ski base material is made of ultra high molecular weight polyethylene having a molecular weight of at least 500,000. After heating, quenching and light tensioning operations, this material exhibits low crystallinity and high transparency characteristics. Such material is ideal for professional high speed skis because of its excellent wax retention quality. The invented ski base material is ideally suited for product-identity purposes because of its outstanding ability to clearly reveal detailed inscriptions placed on the running surface of a ski board.

14 Claims, 1 Drawing Sheet





FIG.1

## SNOW SKI BASE MATERIAL AND SKI BASE MANUFACTURE

This application is a divisional, of application Ser. No. 07/640,860, filed Jan. 14, 1991 now U.S. Pat. No. 5,189,130.

### FIELD OF THE INVENTION

This invention relates to an improved snow ski base material made of ultra high molecular weight polyethylene (UHMWPE) and a quenching method of manufacturing a base (known as a "sole") for high performance snow skis, having improved transparency and wax absorbing capability.

### PRIOR ART

Wear resistant snow ski bases made of UHMWPE group materials have been known, such as those disclosed in Japanese Laid-Open Patent Publications, Sho61-82772 and Sho62-217980, for example.

However, such UHMWPE materials as disclosed in Sho61-82772, for example, often exhibit poor ability to spread wax and even less ability to permit the wax to penetrate into itself, and consequently, such bases lacked fast running capabilities in adverse snow conditions.

### SUMMARY OF THE INVENTION

The purpose of the present invention is to provide a UHMWPE snow ski base material (hereinafter referred to as ski base material) which has high wax absorbing and retaining capabilities.

According to an aspect of this invention, there is provided a UHMWPE ski base material having a molecular weight not less than 500,000 and light transmissivity not less than 10%.

According to another aspect of this invention, there is provided an UHMWPE ski base material having wax absorbing capability of not less than 1.8 mg/cm<sup>2</sup>.

According to still another aspect of this invention, there is provided a method of manufacturing a snow ski base (hereinafter referred to as a ski base) using said UHMWPE material by heating it to a controlled melting state followed by quenching.

### BRIEF DESCRIPTION OF THE DRAWING

FIG. 1 is an angle view of a cross section of a ski board to illustrate its construction.

### DETAILED DESCRIPTION OF THE PRESENT INVENTION

FIG. 1 shows a cross section of a ski board made with the ski base material presented in this invention, and shows a number of components referenced by reference numerals. The reference numeral 1 is a core material, made of foamed resins such as foamed polyurethane and acrylic resins. The core is laminated with top and bottom reinforcing laminations 2, which are made of strip materials made of metals such as high strength aluminum alloys, and non-metals such as glass-fibre or carbon-fibre reinforced polymeric strip materials. The top surface of the above assembly is provided with a decorative component 3, which is further covered with a clear protective layer 4, of thickness 20 to 100 µm, made of urethane or unsaturated polyester resins, so that the decoration is visible. The clear layer 4 is the topmost outer surface of the ski board.

The bottom reinforcing lamination 2 is shown in this figure facing the top of the page and is affixed with said base material 5 of thickness 0.5 to 1.5 mm. The surface thus constructed of said ski base material becomes the running surface 5 in contact with the snow. Therefore, although shown at the bottom of the ski board in this figure, the numeral 6 refers to cosmetic edge protectors, made of aluminum alloys, disposed on the top surface of the ski board when it is being used, and the numeral 7 refers to running edges, made of carbon steels and other hard metallic materials, disposed on the running surface.

The above base material 5 is made of UHMWPE having the molecular weight of not less than 500,000, having melt index not more than 0.01, having density not more than 0.93 g/cm<sup>3</sup> and the degree of crystallinity not more than 55%.

When the ski base is made from an UHMWPE material having the molecular weight not less than 500,000 and light transmissivity not less than 10%, because non-crystalline regions are distributed throughout the base thickness, wax absorbing capability of the base is increased to not less than 1.8 mg per cm<sup>2</sup> of running surface of the base, compared with the conventional similar materials. This is because many regions where crystallization is suppressed, such as amorphous or pracrystalline regions, are distributed throughout from the surface to the inside of the ski base.

The definitions of the light transmissivity and wax absorbing capability will be defined later.

A method of manufacturing the base using such an UHMWPE material will be described next.

A powder of UHMWPE material, of molecular weight not less than 500,000 and preferably not less than 1,000,000 and further having melt index not more than 0.01, is selected from such potential materials as "High-zex Million" made by Mitsui Oil and Chemicals or "Hostallen GUR" made by Hochest Chemicals. The molecular weight referred here is that measured by the viscosity method. This powder is charged into a metal mold and hot pressed to produce a disc-shaped preform. Hot pressing conditions were, for example, pressing at 10 MPa for 5 to 10 minutes at room temperature, followed by pressing at 2 to 5 MPa at temperatures between 200° to 250° C. for 7 to 10 hours, and ending in cooling over a period of 4 to 7 hours while increasing the pressure gradually to 10 MPa.

This disc-shaped preform is subjected to skiving (to peel off a thin layer from the outer periphery) to obtain a thin polyethylene strip having the same width as the preform and a thickness in the range of 0.5 to 2 mm.

The strip is cut into a suitable length for a ski board, and is heated by a suitable method to temperatures in the range of 140° to 150° C. for a period of 10 to 30 minutes. What is required in this processing step is to soften the polyethylene strip sufficiently for the subsequent processing step. Therefore, the choice of heating method could include any one of heating methods such as far-infrared heating, resistive heating, gas flame and high pressure steam. It is desirable to maintain the strip in a horizontal position during heating. It is also desirable to prevent the oxidation of its surface by protecting the strip in between two films of polyethylene telephthalate, Teflon, aluminum foils or by heating the strip in a protective atmosphere such as in inert gas.

In this processing step, if the molecular weight is over 500,000, i.e. its melt index is not more than 0.01, it is possible to prevent its liquefaction and retain the bulk

shape of the UHMWPE material which would just become rubbery under the above specified conditions. The heated strip can then be hung vertically without losing its form entirely.

When all the crystalline phases in the UHMWPE strip have been melted or become amorphous and transparent, the strip is taken out of the furnace and is quenched immediately by immersing it in an quenching medium such as cold water. The quenching medium can also be a mixture of alcohol and dry ice or liquid nitrogen, or other low temperature liquid medium which has high heat capacity. The cooling rate should be no less than 100° C./s., and preferably in excess of 200° C./s. in order that the amorphous phase will increase thus leading to high absorbing capability of wax. Quenching methods include placing a quenching bath, large enough to contain the strip, beside the heating furnace so that the strip can be immersed in the bath within one second of taking it out of the furnace.

Such rapid cooling of heated UHMWPE strip promotes retention of the amorphous state of the softened material and suppresses crystallization during cooling.

The distortions of the UHMWPE strip created by quenching stresses are corrected by reheating the quenched strip to 70° to 90° C., and stretching the strip in the longitudinal direction for several minutes, and cooling it under tension.

The base material thus produced is further subjected to such surface activation steps as flame treatment so that adhesive property of the base material will improve, and after this treatment, the surface layer of the base material is removed slightly to finish it as the running surface. Then, bonding among the base materials, the reinforcements 2, and the core material 1 is carried out by the conventional techniques to produce a ski board.

The crystalline phase through the thickness of the UHMWPE base material thus obtained has been kept to a minimum from the surface to the inside by the combined action of controlled heating and rapid quenching, and the base made of such a material has superior transparency and light transmissivity compared with the conventional sintered ski base. In the present invention, the acceptable base material is defined as those having light transmissivity of not less than 10%.

Light transmissivity is based on the wave length of 517 nm transmitted through an UHMWPE sample of 1.00 mm thickness. The method of measurement is as follows. A sample for light transmission measurement is prepared by polishing and spreading silicon oil on the two surfaces of a quenched strip, and covering the two surfaces with microscope slide glasses so as to fill the capillary space between the sample and the slide glass with the silicone oil. This is to avoid the light scattering effects due to the presence of irregularities on the UHMWPE sample surface. A comparative reference is also made in the form of a sandwiched slide glasses filled with the same silicon oil. Light transmission through the sample is measured with a spectrophotometer at the wave length of 517 nm, and the transmissivity at the exact thickness of 1.00 mm is calculated according to Lambert's Law.

The UHMWPE material having light transmissivity of not less than 10% has good transparency and the ski base prepared from such a material provides excellent visibility of the patterns/printing 8 conferred on the surface of the reinforcing laminations 2 through the transparent ski base material 5 adapted to become the

running surface, as depicted in FIG. 1. Because the base is clear, even fine details can be seen vividly on the ski base, compared with the conventionally prepared ski base materials.

Furthermore, the base materials made of UHMWPE having not less than 10% transmissivity has a superior wax absorbing capability as represented by a figure of 1.8 mg per one cm<sup>2</sup> of the running surface.

As demonstrated in the foregoing preferred embodiment, the ski base prepared by heating and quenching UHMWPE material according to this invention has not less than 10% light transmissivity as the crystallization is suppressed from the surface to the inside of the base and provides outstanding transparency and wax absorbing capability.

Therefore, the skis equipped with the invented ski base require waxing less often and are able to provide excellent performance advantages, over other skis with a conventional ski base, when skiing on wet snow, new snow, long distance skiing and other adverse conditions in which waxing could provide the critical winning edge.

Furthermore, because the base has good transparency, it provides an excellent visibility of the decorative patterns and inscriptions thereon, thus furnishing outstanding opportunity for product-identification.

Wax absorbing capability is measured as follows. A sample of UHMWPE of 40 mm × 25 mm is weighed to obtain its initial weight ( $M_0$ , mg) and the surface area measurements ( $A$ , cm<sup>2</sup>) are made. It is then immersed in molten paraffin, having a melting range of 52° to 54° C. (DAB 9 or DAB 8, for example Merk No. 7152), maintained at 110° C. ± 2° C. After ten minutes of immersion, the sample is taken out and wiped immediately with absorbing cloth or paper. The sample is allowed to cool for ten seconds and then is immersed in a solution of diethylether for ten seconds to remove traces of surface wax. The cleaned sample is weighed to determine the new sample weight ( $M$ ) and the amount of wax absorbed  $W$  is calculated according to the following formula.

$$W = (M - M_0) / A \text{ (mg/cm}^2\text{)}$$

It has been found that those UHMWPE samples, exhibiting light transmission values of not less than 10%, have high values of wax absorbing capability. It is believed that these samples have low degrees of crystallinity and high degrees of amorphousness, and because the amorphous material has good miscibility with wax, the wax absorbing capability of such amorphous materials is increased.

It has furthermore been found that those samples of UHMWPE having not less than 10% light transmissivity show low degrees of crystallinity of around 55% or less.

The degree of crystallinity is determined from the density of UHMWPE as follows. The formula for the degree of crystallinity of a sample having a density  $d$  is given by the values of the density of crystalline phases  $d_c$  and amorphous phase  $d_a$  respectively according to the following formula.

$$\text{DEGREE OF CRYSTALLINITY} \\ (\%) = [d_c(d - d_a)] / [d(d_c - d_a)] \times 100$$

where the values of  $d_c$  and  $d_a$  are taken as 1.000 g/cm<sup>3</sup>, and 0.856 g/cm<sup>3</sup>, respectively. Therefore, a density

value can be determined readily on a small sample piece cut out of a heat treated strip by using a density gradient tube (i.e. a tube containing stratified layers of liquids of varying densities).

In the following, some cases of preferred embodiments are presented.

#### A First Preferred Embodiment

An UHMWPE preform having a molecular weight of 4,000,000 was made into a test sample measuring 10 cm width  $\times$  200 cm length  $\times$  1.0 mm thickness by skinning. This material exhibited 62.6% crystallinity, 1.54 mg/cm<sup>2</sup> wax absorbing capability and 6% light transmissivity.

The above material was made into a ski base material by heating for 20 minutes at 150° C., quenching in water at 10° C. and shaping using light tensioning at 60° C. This ski base material exhibited 51.7% crystallinity, 0.925 g/cm<sup>3</sup>, 2.18 mg/cm<sup>2</sup> wax absorbing capability and increased its light transmissivity to 33.7%.

#### A Second Preferred Embodiment

An UHMWPE preform having a molecular weight of 6,000,000 was made into a ski base material by using the same procedure as in the first preferred embodiment. The untreated material exhibited 56.8% crystallinity, 1.58 mg/cm<sup>2</sup> wax absorbing capability and 7.01% light transmissivity.

The above material was heat treated at 140° C. for 30 minutes and quenched in water at 20° C. This material was treated by the same shaping procedure as in the first preferred embodiment.

The ski base material thus prepared exhibited 50.7% crystallinity, 0.923 g/cm<sup>3</sup>, 2.01 mg/cm<sup>2</sup> wax absorbing capability and improved its light transmissivity to 18.5%.

#### A Third Preferred Embodiment

An UHMWPE preform having a molecular weight of 8,000,000 was made into a ski base material by using the same procedure as in the first preferred embodiment. The untreated material exhibited 58.4% crystallinity, 1.47 mg/cm<sup>2</sup> wax absorbing capability and 8.5% light transmissivity.

The above material was heat treated at 160° C. for 10 minutes and quenched in water at 0° C. This material was shaped by the same shaping procedure as in the first preferred embodiment.

The ski base material thus prepared exhibited 50.9% crystallinity, 0.925 g/cm<sup>3</sup>, 2.40 mg/cm<sup>2</sup> wax absorbing capability and improved its light transmissivity to 16.2%.

#### Comparative Example No. 1

A ski base material of 1.5 mm thickness was made by extruding an UHMWPE having a molecular weight of 100,000. The crystallinity was 72.6%, its wax absorbing capability was 1.57 mg/cm<sup>2</sup> and light transmissivity was 1.4%.

#### COMPARATIVE EXAMPLE NO. 2

An UHMWPE material having a molecular weight of 200,000 was made into a ski base material by the process described in the first preferred embodiment.

The above material was heat treated at 150° C. for 20 minutes, it was then discovered that quenching cannot be performed as the material had become too fluid.

What is claimed is:

1. A method of making a snow ski base material, wherein said base material consists essentially of ultra high molecular weight polyethylene having a molecular weight of 500,000 to 8,000,000, a light transmissivity of 10 to 33.7%, a density of not more than 0.93 g/cm<sup>3</sup> and a degree of crystallinity quality of not more than 55%, and is treated by a two-step process of heating to a controlled melting state followed by quenching under normal atmospheric pressure, said method further including the steps of charging the ultra high molecular weight polyethylene into a metal mold and hot pressing the ultra high molecular weight polyethylene therein.

2. A method of making a snow ski base material according to claim 1, wherein said ski base material is quenched at a rate in excess of 100° C. per second.

3. A method of making a snow ski base material consisting essentially of ultra high molecular weight polyethylene having a molecular weight of 500,000 to 8,000,000, a light transmissivity of 10 to 33.7%, a density of not more than 0.93 g/cm<sup>3</sup> and a degree of crystallinity quality of not more than 55%, and comprising the steps of:

charging the ultra high molecular weight polyethylene into a metal mold;  
hot pressing the ultra high molecular weight polyethylene in the metal mold;  
heating the ultra high molecular weight polyethylene to a controlled melting state; and  
quenching the melted ultra high molecular weight polyethylene in a quenching medium under normal atmospheric pressure to produce a snow ski base material having a density of not more than 0.93 g/cm<sup>3</sup> and a wax absorbing capability of 1.8 to 2.4 mg per one square centimeter of running surface area.

4. A method of making a snow ski base material according to claim 3, further including a step of:

quenching the ski base material at a rate in excess of 100° C. per second.

5. A method of making a snow ski base material according to claim 3, wherein said step of pressing is performed at 10 MPa at room temperature, followed by pressing at 2 to 5 MPa at temperatures ranging from 200°-250° C., and further comprising the step of:

cooling the pressed ultra high molecular weight polyethylene while increasing pressure to 10 MPa.

6. A method of making a snow ski base material according to claim 3, further including the step of:

skiving the pressed ultra high molecular weight material to produce a polyethylene strip having a thickness of 0.5 mm to 2 mm.

7. A method of making a snow ski base material according to claim 6, wherein said step of heating is performed at temperatures ranging from 140° C. to 150° C.

8. A method of making a snow ski base material according to claim 7, wherein said step of heating is performed using far-infrared heating, resistive heating, gas flame or high pressure steam.

9. A method of making a snow ski base material according to claim 8, wherein to prevent oxidation of a surface of the ultra high molecular weight polyethylene during said heating step, said heating step further includes the step of:

protecting the polyethylene strip by placing the polyethylene strip between two films of polyethylene telephthalate, teflon, aluminum foils or by heating the strip in a protective atmosphere.

10. A method of making a snow ski base material according to claim 9, wherein said step of quenching further includes the steps of:

immersing the polyethylene strip in a quenching medium which includes at least one of cold water, alcohol or liquid nitrogen, with a cooling rate greater than 100° C./s. 5

11. A method of making a snow ski base material according to claim 10, further including the step of:

reheating the polyethylene strip after said step of quenching; and 10

15

stretching the reheated strip and cooling the stretched strip under tension.

12. A method of making a snow ski base material according to claim 11, further including the step of: subjecting the quenched polyethylene strip to flame treatment to improve an adhesive property of the material.

13. A method of making a snow ski base material according to claim 1, wherein said molecular weight is measured using a viscosity measurement technique.

14. A method of making a snow ski base material according to claim 3, wherein said molecular weight is measured using a viscosity measurement technique.

\* \* \* \* \*

20

25

30

35

40

45

50

55

60

65